

732,226

No. 732,226.

Patented June 30, 1903.

## UNITED STATES PATENT OFFICE.

JOHANN SENFT, OF VIENNA, AUSTRIA-HUNGARY.

## COMPOSITION OF PAINTING-CEMENT.

SPECIFICATION forming part of Letters Patent No. 732,226, dated June 30, 1903.

Application filed August 20, 1902. Serial No. 120,381. (No specimens.)

106-79

*To all whom it may concern:*

Be it known that I, JOHANN SENFT, a subject of the Emperor of Austria-Hungary, residing at Seidelgasse No. 12, Vienna III, in the 5 Province of Lower Austria and Empire of Austria-Hungary, have invented a new and useful Composition of Painting-Cement for Wood, Metals, and Brickwork, of which the following is a specification.

10 My invention relates to the manufacturing of a painting-cement which can be used with equally good success for coating wood, metals, and brickwork, which has the essential advantage before all other cements in use that 15 putting with the spatula is avoided, a tedious work requiring much time and skill, but necessary with any method of varnishing or painting at present in use.

In order to manufacture the said painting-cement, the following ingredients are to be 20 mixed in about the given proportions, viz: twenty-five per cent. white lead, 12.5 per cent. white or pure litharge, 3.75 per cent. polishing-varnish, composed of fossil resins, (as copal or amber,) linseed-oil, and turpentine, 25 7.5 per cent. bone-glue, 2.5 per cent turpentine-oil, 2.5 per cent. potassium silicate, ten per cent. siccative, fifteen per cent. rock-lime, and 21.25 per cent. water. This mixture forms 30 a pulp after having been ground on the color-

grinder and may be diluted with water at discretion. For a moderate coat with the brush about one kilogram suffices for ten square meters.

This composition is a good medium for filling up the pores and renders the ground color superfluous, as it has itself enough covering capacity and working becomes therefore quicker and cheaper.

This cement is drying very quickly, becomes quite hard, but is not brittle, so that it does not come off. It is fireproof and is easily polished off with some sandpaper.

What I claim, and desire to secure by Letters Patent, is—

The herein-described composition of painting-cement quickly drying and rendering the ground color superfluous, consisting of white lead, pure litharge, polishing-varnish, bone-glue, turpentine-oil, potassium silicate, siccative, rock-lime and water in the proportions specified which ingredients are to be ground to pulp in a color-grinder.

In witness whereof I have hereunto set my hand in presence of two witnesses.

JOHANN SENFT.

Witnesses:

ALFRED SENFT,  
ALVESTO S. HOGUE.